

## UNITED STATES PATENT OFFICE.

HERMANN KAMBACH, OF BERLIN-CHARLOTTENBURG, GERMANY.

## ARTIFICIAL ASPHALT AND METHOD OF MAKING A STABLE MIXTURE THEREOF WITH STONY MATERIAL.

No Drawing.

Application filed May 26, 1921. Serial No. 472,923.

*To all whom it may concern:*

Be it known that I, HERMANN KAMBACH, a citizen of the German Empire, residing at Berlin-Charlottenburg, Germany, have invented certain new and useful Improvements in Artificial Asphalt and Methods of Making a Stable Mixture Thereof with Stony Material, of which the following is a specification.

10 My invention refers to asphalt for road making and the like and its particular object is a novel bitumen like product adapted to replace natural asphalt and to re-generating broken natural asphalt. My invention 15 furthermore refers to a method for making a composition of the novel product with stony material in order to form a stable mass for road making.

Owing to its low wear and the great saving 20 of the vehicles and so on the so called compressed asphalt has up till now been made use of in many instances in road making, for pavements, side walks and the like. The foreign asphalt imported as a rule from 25 Sicily has up till now formed the only raw-material, which has not been replaced by others.

The novel product according to the present invention, being made of raw-materials 30 obtainable in every coal-producing country and equalling the asphalt imported from abroad as far as road making and the like are concerned offers the great advantage of rendering the national industry independent 35 from foreign countries, the more so as the price of the novel product is considerably lower than that of Sicilian asphalt.

The novel mass essentially consists of coal tar pitch and tar, anthracene oil being 40 added, if necessary, and a vegetable oil such as linseed oil, or a plurality of liquid oils such as a mixture of linseed oil and rape seed oil.

The difference between the freezing point 45 and melting point of a bitumen-like mass composed for instance of 5 parts by weight of linseed oil, 5 parts rape seed oil, 70 parts coal tar pitch, 15 parts anthracene oil and 15 parts coal tar amounts to about 60° C. According to climatic conditions these 50 points may be raised or lowered by varying the percentage of tar or its products. In this manner the novel mass warrants absolute solidity regardless of any change of temperature and the greatest resistibility

against the action of cold and heat, thus offering a most perfect substitute for Sicilian asphalt.

Old broken natural asphalt is revived by an addition of one or two per cent of my 60 novel mass to such an extent as to be at least equal to fresh asphalt.

In order to obtain artificial compressed asphalt according to the present invention I may for instance proceed as follows: To 65 a mixture of 5 parts linseed oil, 5 parts rape seed oil, 70 parts coal tar pitch, 15 parts anthracene oil and 15 parts coal tar there are added for instance 1000 parts stone meal or the like. This mixture is heated 70 to about 170—175° C. and can then be compressed. Its specific weight is about 2.2—2.3. The compressed mass is absolutely impervious to water and also water proof. It will resist the highest pressure occurring in road traffic. 75

By heating the bitumen-like mass described in the first instance with the stony materials mentioned above to about 100° C. a stable asphalt mass is obtained which 80 may be kept in store for subsequent use and need only be heated to about 170° C. (preferably by aid of steam) and then be compressed.

## I claim:

1. As a novel product for making compressed paving material and for regenerating broken natural asphalt, a mixture of coal tar pitch, coal tar, anthracene oil and a vegetable oil. 85

2. As a novel product for making compressed paving material and for regenerating broken natural asphalt, a mixture of coal tar pitch, coal tar, anthracene oil and vegetable oils of different kinds. 90

3. As a novel product for making compressed paving material, a mixture of coal tar pitch, coal tar, anthracene oil and a vegetable oil with finely comminuted stony material. 95

4. As a novel product for making compressed paving material, a mixture of coal tar pitch, coal tar, anthracene oil and vegetable oils of different kinds with finely comminuted stony material. 100

5. As a novel product, a mixture comprising 70 parts coal tar pitch, 15 parts anthracene oil, 15 parts coal tar and 10 parts linseed oil. 105

6. As a novel product, a mixture compris- 110

ing 70 parts coal tar pitch, 15 parts anthracene oil, 15 parts coal tar and 5 parts linseed oil and 5 parts rape seed oil.

7. As a novel product, a mixture comprising 70 parts coal tar pitch, 15 parts coal tar, 15 parts anthracene oil, 10 parts linseed oil and about 1000 parts of finely comminuted stony material.

8. As a novel product, a mixture comprising 70 parts coal tar pitch, 15 parts coal tar, 15 parts anthracene oil, 5 parts linseed oil, 5 parts rape seed oil and about 1000 parts of finely comminuted stony material.

9. The method which consists in heating coal tar pitch, coal tar, anthracene oil and a vegetable oil with finely comminuted stony material to about 100° C.

10. The method which consists in heating coal tar pitch, coal tar, anthracene oil and vegetable oils of different kinds with finely comminuted stony material to about 100° C.

In testimony whereof I affix my signature.

HERMANN KAMBACH.

Witnesses:

PAUL FISCHER,  
HANS VON NICKEN.